

# United States Patent

[19]

Lindstedt

[11] 3,888,704

[45] June 10, 1975

[54] **METHODS OF TREATING HARDENING OIL BEFORE USE BY ADDING A MIXTURE OF ETHOXYLATED ACYCLIC COMPOUNDS AND FILM-FORMING ACYCLIC COMPOUNDS**

[75] Inventor: **Per Olof Lindstedt**, Molndal, Sweden

[73] Assignee: **Olof Lindstedt & Co. AB**, Molndal, Sweden

[22] Filed: **Feb. 20, 1974**

[21] Appl. No.: **444,223**

[52] U.S. Cl. .... **148/29; 252/73; 252/77; 252/79**

[51] Int. Cl. .... **B23k 35/24**

[58] Field of Search .... **148/29, 28, 27, 143, 20.6, 148/18; 252/74, 75, 77, 79, 73, 76**

[56]

## References Cited

### UNITED STATES PATENTS

|           |         |                    |          |
|-----------|---------|--------------------|----------|
| 3,192,165 | 6/1965  | Fields et al. .... | 252/79   |
| 3,224,910 | 12/1965 | McEwen.....        | 148/143  |
| 3,281,288 | 10/1966 | Carver et al. .... | 148/20.6 |
| 3,340,193 | 9/1967  | Fields et al. .... | 252/79   |

Primary Examiner—Walter R. Satterfield

[57]

## ABSTRACT

A mixture consisting of ethoxylated acyclic compounds as emulsifiers, acyclic compounds as film-forming agents and possibly antioxidants and corrosion inhibitors, is added to a mineral-oil based hardening oil.

5 Claims, No Drawings

**METHODS OF TREATING HARDENING OIL  
BEFORE USE BY ADDING A MIXTURE OF  
ETHOXYLATED ACYCLIC COMPOUNDS AND  
FILM-FORMING ACYCLIC COMPOUNDS**

The use of liquids for the hardening of metals is well known. For example, metallic objects can be cooled rapidly by immersing them in water or oil. Immersion in oil often produces a milder and a more even effect since the occurrence of stress within the material is avoided.

The oils used must be stable at the temperatures in question and often paraffin- or naphthalene-based mineral oils or mixtures thereof are used, if desired with additives included.

After the immersion the oil should be removed from the metal surface. This can be done by alkaline washing or by treatment with solvents, such as chlorinated hydrocarbons. Another possibility is to add an emulsifier to the hardening oil. In that case the oil after hardening is removed from the material by flushing with water.

The emulsifiers used in the latter case must possess a high emulsifying capacity and be thermostable so that no decomposition products are created which could have an injurious effect on the surface of the metal. The emulsifiers must also be relatively insensitive to the hardness and pH of the water, so that immersion or spraying with water does not result in precipitations which could be harmful to the metal surface.

From the point of view of environmental preservation it is important that the emulsifiers chosen can be decomposed biologically, so that they are incapable of causing any damage.

It has been found that certain ethoxylated acyclic compounds, viz. ester, alkyl ether, fatty acid amide and alkylamine-ethylene oxide adducts, satisfy the above-mentioned requirements. Such acyclic compounds contain 8-20 C-atoms in straight or branched alkyl chains which can be saturated or unsaturated, or mixtures thereof, and at least one active H-atom. The following are suitable compounds:

- a. Fatty acids containing 10-20 C-atoms.
- b. Alkanols, primary or secondary, such as cetyl alcohol, oleyl/cetyl alcohol, tridecyl alcohol,  $C_8-C_{16}$  alkanols,  $C_{10}-C_{20}$  alkanols, etc.
- c. Carboxylic acid amides, such as palmitic acid mono or diethanolamide, oleic acid- lauric acid mono- or diethanol-amide, etc.
- d. Primary, secondary or tertiary alkyl amines and alkyl polyamines, such as lauryl amine, lauryl oleyl amine, tallow amine, tallow propylene diamine, etc.

After the building up of ethylene oxide these products contain 2-15, preferably 2-8, ethylene oxide units in the hydrophilic part.

It is of the utmost importance that a thin film be left on the surface of the metal after the removal of the hardening oil. In order to achieve this a compound which is, in itself, neither soluble in nor dispersible by water, is added to the oil, in addition to the emulsifier. In order to make this film adhere well to the metal surface it should contain one or more  $OH-$ ,  $-CONH_2$ , or  $NH_2$ -groups. This oil film protects the surface against corrosion.

An addition of this type to the hardening oil acts also as solubilizer for the ethoxylated emulsifier, thereby

ensuring a better distribution of the latter in the mineral oil.

Suitable film-forming additives are acyclic compounds or mixtures thereof with straight or branched, saturated or partially saturated alkyl chains containing 10-26 C-atoms and at least one polar group, such as  $OH$ ,  $-CONH_2$ , or  $NH_2$ -groups.

Suitable compounds are: fatty acid esters, cetyl oleyl alcohol, tridecyl alcohol, stearyl alcohol, alkanols with 10-16 C-atoms, lauric acid mono-ethanolamide, lauryl amine, tallow amine, tallow diamine, etc.

It is advisable to mix the emulsifier with the film-forming additive before adding it to the mineral oil. In this case suitable mixing proportions are: 60-95 percent ethoxylated acyclic compounds and 40-5 percent film-forming additives. This mixture is added to the oil in an amount of 1-10 percent, preferably 2-5 percent, by weight of the oil.

Also other additions may prove appropriate. Thus, 20 the addition of an antioxidant, such as dibutyl phenol or dibutylmethyl phenol, may be considered. The addition ratio is approximately 0.5-1 percent by weight of the oil.

In certain cases the addition of a corrosion inhibitor 25 may also be required. An acyclic amine compound containing 10-20 C-atoms, such as cetylamine or lauryl diamine, can be used for this purpose, the addition ratio being 0.5-1.5 percent by weight of the oil.

The invention will be illustrated by the following Examples in which two mineral oils were used, i.e. one paraffin-based oil with 2.1 E°/50°C viscosity and one naphthalene-based oil with 7.5 E°/50°C viscosity.

The mineral oils were mixed with an emulsifier or an emulsifier mixture in the proportion 97:3 percent by weight. The mineral oil containing the emulsifier or emulsifier mixture was then mixed with water in the proportion 5 parts by weight of mineral oil + emulsifier to 95 parts by weight of water.

In certain cases, the mineral oil + emulsifier or emulsifier mixture were, before mixing, heated for 18 hours up to 180°C. After the emulsifier-bearing mineral oil had been mixed with water, the emulsion was left to stand for one-half hour, after which the surface creaming was measured; it is stated as a percentage of the emulsion.

A very important factor is the solubility of the emulsifier, or emulsifier mixture, in the mineral oil. In order to arrive at a good, even emulsification and, above all, a long storage life, the emulsifier or emulsifier mixture should be clearly dissolved in the mineral oil. To allow comparison of the results obtained, the content of the emulsifier or emulsifier mixture in the mineral oil was at all times maintained at 3 percent by weight.

**EXAMPLE 1**

97 Parts by weight of a paraffin-based oil were mixed with 3 parts by weight of an emulsifier mixture containing 90 percent lauryl alcohol polyglycol ether with 3 mols of ethylene oxide per mol of lauryl alcohol, and 10 percent 50/55 oleyl/cetyl alcohol. A clear and translucent oil mixture was obtained. After mixing the emulsion, creaming amounted to 3-4 percent after one-half h.

With another, identically composed sample a heat resistance test was carried out; after formation of the emulsion this oil has showed 3-4 percent creaming after one-half h. Thus, the emulsifying capacity of the

oil mixture was not reduced by heating it for 18 h to 180°C.

For purposes of comparison an ethoxylated nonyl phenol of the same proportions as mentioned above containing 6 mols of ethylene oxide was added to the paraffin-based oil. This mixture was, however, cloudy, unlike the preceding one which was completely clear. Cloudiness means, as has been already mentioned, that there is a great risk that the emulsion will separate under storage.

As regards the emulsifying capacity both before and after heating, which was carried out in the same way as mentioned above, creaming amounted to 3-4 percent in both cases.

#### EXAMPLE 2

3 Parts by weight of an emulsifier mixture containing 90 percent lauryl alcohol polyglycol ether with 3 mols of ethylene oxide per mol of lauryl alcohol and 10 percent of a mixture of saturated, straight fatty alcohols containing 12 and 14 carbon atoms, respectively, were added to 97 parts by weight of paraffin-based oil. This emulsifier mixture also dissolved completely clearly in the paraffin-based oil. The emulsifying capacity was approximately the same as was mentioned earlier, i.e. creaming amounted to 3-4 percent.

#### EXAMPLE 3

3 Parts by weight of an emulsifier mixture containing 90 percent lauryl alcohol polyglycol ether with 3 mols of ethylene oxide per mol of lauryl alcohol and 10 percent coconut fatty acid diethanolamide were added to 97 parts by weight of paraffin-based oil. The emulsifier mixture dissolved completely clearly in the paraffin-based oil. The emulsifying capacity was the same as was mentioned in the preceding Examples.

#### EXAMPLE 4

97 Parts by weight of a paraffin-based oil were mixed with 3 parts by weight of an emulsifier mixture containing 90 percent oleyl amine polyglycol ether with 7 mols of ethylene oxide per mol of oleyl amine and 10 percent 50/55 oleyl/cetyl alcohol. The emulsifier mixture dissolved clearly in the mineral oil.

#### EXAMPLE 5

97 Parts by weight of a naphthene-based oil were mixed with 3 parts by weight of an emulsifier mixture containing 90 percent lauryl alcohol polyglycol ether with 3 mols of ethylene oxide per mol of lauryl alcohol and 10 percent oleyl/cetyl alcohol.

The oil mixture dissolved completely clearly in the mineral oil. As was mentioned in Example 1, the emulsifying capacity was tested first with the abovementioned oil mixture per se and secondly with the abovementioned oil mixture heated for 18 h to 180°C. In both cases the emulsions indicated 1-2 percent creaming after one-half h.

For purposes of comparison, a nonyl phenol polyglycol ether containing 6 mols of ethylene oxide per mol of nonyl phenol was used as an emulsifier also in this case. This product, in the proportions 97 parts by weight naphthene-based oil to 3 parts by weight emulsifier, was not clearly soluble in the mineral oil. The emulsifying capacity, tested as described previously, was 1-2 percent both before and after heating.

#### EXAMPLE 6

97 Parts by weight of a naphthene-based oil were added to 3 parts by weight of an emulsifier mixture containing 90 percent lauryl alcohol polyglycol ether with 3 mols of ethylene oxide per mol of lauryl alcohol and 10 percent coconut fatty acid diethanol amide. The product dissolved clearly in the naphthene-based oil, and had the same emulsifying capacity as the emulsifier mixture mentioned in Example 5.

#### EXAMPLE 7

97 Parts by weight of a paraffin-based oil were mixed with 3 parts by weight of an emulsifier mixture containing 90 percent oleyl cetyl polyglycol ether with 5 mols of ethylene oxide per mol of oleyl/cetyl alcohol and 10 percent of a fatty alcohol mixture with 20 or more C-atoms in the alkyl group. The emulsifier mixture dissolved almost clearly in the oil. A 5 percent emulsion indicated 4.5 percent creaming one-half h after mixing and one-half h after heat treatment.

The same test carried out with naphthene-based oil gave a clear solution of the emulsifier mixture in the mineral oil and the emulsion indicated 2 percent creaming before and after heat treatment.

Thus, the emulsifying capacity was not impaired either in paraffin-based or naphthene-based oil.

#### EXAMPLE 8

97 Parts by weight of paraffin-based oil were mixed with 3 parts by weight of an emulsifier mixture containing 79 percent tallow diamine polyglycol ether with 3 mols of ethylene oxide per mol of tallow diamine, 20 percent oleyl/cetyl alcohol, 1 percent tallow diamine as a corrosion inhibitor. The emulsifier mixture was clearly soluble in the mineral oil and gave a fine emulsion. After one-half h before and after heating creaming amounted to 3 percent.

The same test in the naphthene-based oil gave a clear solution of the emulsifier mixture in the mineral oil, a fine emulsion, and 1 percent cream before and after heating.

Thus, the emulsifying capacity showed no change either in paraffin-based or in naphthene-based oil.

#### EXAMPLE 9

97 Parts by weight of paraffin-based oil were mixed with 3 parts by weight of an emulsifier mixture containing 70 percent ethoxylated oleic acid diethanolamide with 10 mols of ethylene oxide per mol of oleic acid diethanolamide and 30 percent oleyl/cetyl alcohol. The emulsifier mixture was clearly soluble in the oil and resulted in rapid emulsion, and the emulsion produced 5 percent cream + oil before and after heating.

The test with the same emulsifier mixture in naphthene-based oil gave an opaque solution of the emulsifier in the oil and the emulsion produced 4 percent cream + oil before and after heating.

The emulsifying capacity of the mixture was inferior to that of the preceding examples; the heating, however, did not result in any deterioration.

#### EXAMPLE 10

97 Parts by weight of paraffin-based oil were mixed with 3 parts of an emulsifier mixture containing 88 percent lauryl alcohol polyglycol ether, 10 percent oleyl/cetyl alcohol and 2 percent stearyl amine. The emulsi-

fier mixture dissolved clearly in the mineral oil and the emulsion produced, before heating, 4.5 percent cream + oil and, after heating, 5 percent cream.

The same emulsifier mixture in naphthene-based oil gave a clear solution and the emulsion produced, before and after heating, 3.5 percent cream.

#### EXAMPLE 11

97 Parts by weight of paraffin-based oil were mixed with 3 parts of an emulsifier mixture containing 90 percent ethoxylated coconut fatty acid mono-ethanolamide with 2 mols of ethylene oxide per mol of coconut fatty acid mono-ethanolamide and 10 percent olive oil. The emulsifier mixture dissolved almost clearly in the oil, gave a fine emulsion and produced, before and after heating, 4.5 percent cream.

The same emulsifier mixture was almost clearly soluble in naphthene-based oil and the emulsion indicated before and after heating 3.5 percent creaming.

#### EXAMPLE 12

97 Parts by weight of naphthene-based oil were mixed with 3 parts by weight of an emulsifier mixture containing 67 percent oleic acid polyglycol ester and 33 percent oleyl amine. The oleic acid polyglycol ester contained 6 mols of ethylene oxide per mol of oleic acid. The emulsifier mixture dissolved opaquely in the oil and the emulsion indicated, before heating, 2 percent and, after heating, 2.5 percent creaming.

#### EXAMPLE 13

97 Parts by weight of paraffin-based oil were mixed with 3 parts by weight of an emulsifier mixture containing 67 percent oleic acid polyglycol ester with 6 mols of ethylene oxide per mol of oleic acid and 33 percent coconut fatty diamine. The emulsifier mixture dissolved opaquely in the oil and gave a fine emulsion indicating, before heating, 4 percent and, after heating, 4.5 percent creaming.

#### EXAMPLE 14

97 Parts by weight of paraffin-based oil containing 1 percent by weight oleyl amine as a corrosion inhibitor were mixed with 3 parts by weight of an emulsifier mixture containing 90 percent oleic acid polyglycol ester with 6 mols of ethylene oxide per mol of oleic acid and 10 percent oleyl/cetyl alcohol. The emulsifier mixture gave an opaque solution in the mineral oil and a fine emulsion indicating 4.5 percent creaming before and after heating.

97 Parts by weight of naphthene-based oil containing 1 percent by weight of coconut fatty diamine as a corrosion inhibitor were added to 3 parts by weight of the same emulsifier mixture. The dissolved opaquely in the oil and gave a fine emulsion indicating 2 percent creaming before and after heating.

Thus, by adding a corrosion inhibitor directly to the oil and by heating, the emulsifying capacity did not deteriorate.

What I claim and desire to secure by Letters Patent is:

1. A method of improving a mineral oil-based oil for use in cooling metallic objects by rapidly immersing said objects in said oil, said method comprising adding to said oil 1-10 percent, by weight of said oil, of a mixture consisting of:

A. 60-95 percent by weight of an emulsifier, said emulsifier being a biodegradable, ethoxylated, acyclic compound selected from the group consisting of esters, alkyl ethers, fatty acid amides and alkylamine-ethylene oxide adducts, wherein said compound contains 8-20 carbon atoms in alkyl groups and 2-15 hydrophilic, ethylene oxide units; and

B. 40-5 percent by weight of a C<sub>10</sub>-C<sub>26</sub>, film-forming, acyclic compound selected from the group consisting of esters, alcohols, amides and amines, said film-forming compound being neither soluble in nor dispersible by water.

2. A method of improving a mineral oil-based oil for use in cooling metallic objects by rapidly immersing said objects in said oil, said method comprising adding to said oil 1-10 percent, by weight of said oil, of a mixture consisting of:

A. 60-95 percent by weight of an emulsifier, said emulsifier being a biodegradable, ethoxylated, acyclic compound selected from the group consisting of esters, alkyl ethers, fatty acid amides and alkylamine-ethylene oxide adducts, wherein said compound contains 8-20 carbon atoms in alkyl groups and 2-15 hydrophilic, ethylene oxide units;

B. 40-5 percent by weight of a C<sub>10</sub>-C<sub>26</sub>, film-forming, acyclic compound selected from the group consisting of esters, alcohols, amides and amines, said film-forming compound being neither soluble in nor dispersible by water; and

C. an antioxidant selected from the group consisting of dibutyl phenol and dibutyl methyl phenol.

3. A method of improving a mineral oil-based oil for use in cooling metallic objects by rapidly immersing said objects in said oil, said method comprising adding to said oil 1-10 percent, by weight of said oil, of a mixture consisting of:

A. 60-95 percent by weight of an emulsifier, said emulsifier being a biodegradable, ethoxylated, acyclic compound selected from the group consisting of esters, alkyl ethers, fatty acid amides and alkylamine-ethylene oxide adducts, wherein said compound contains 8-20 carbon atoms in alkyl groups and 2-15 hydrophilic, ethylene oxide units;

B. 40-5 percent by weight of a C<sub>10</sub>-C<sub>26</sub>, film-forming, acyclic compound selected from the group consisting of esters, alcohols, amides and amines, said film-forming compound being neither soluble in nor dispersible by water;

C. an antioxidant selected from the group consisting of dibutyl phenol and dibutyl methyl phenol; and

D. a corrosion inhibitor selected from the group consisting of C<sub>10</sub>-C<sub>20</sub> acyclic amines.

4. A method of improving a mineral oil-based oil for use in cooling metallic objects by rapidly immersing said objects in said oil, said method comprising adding to said oil 2-5 percent by weight of said oil, of a mixture consisting of:

A. 60-95 percent by weight of an emulsifier, said emulsifier being a biodegradable, ethoxylated, acyclic compound selected from the group consisting of esters, alkyl ethers, fatty acid amides and alkylamine-ethylene oxide adducts, wherein said compound contains 8-20 carbon atoms in alkyl groups and 2-15 hydrophilic, ethylene oxide units; and

B. 40-5 percent by weight of a C<sub>10</sub>-C<sub>26</sub>, film-forming, acyclic compound selected from the group consisting of esters, alcohols, amides and amines, said

film-forming compound being neither soluble in nor dispersible by water.

5. A method of improving a mineral oil-based oil for use in cooling metallic objects by rapidly immersing said objects in said oil, said method comprising adding to said oil 1-10 percent, by weight of said oil, of a mixture consisting of:

A. 60-95 percent by weight of an emulsifier, said emulsifier being a biodegradable, ethoxylated, acyclic compound selected from the group consisting of:

15.

20.

25.

30.

35.

40.

45.

50.

55.

60.

65.

of esters, alkyl ethers, fatty acid amides and alkylamine-ethylene oxide adducts, wherein said compound contains 8-20 carbon atoms in alkyl groups and 2-8 hydrophilic, ethylene oxide units; and

B. 40-5 percent by weight of a C<sub>10</sub>-C<sub>26</sub>, film-forming, acyclic compound selected from the group consisting of esters, alcohols, amides and amines, said film-forming compound being neither soluble in nor dispersible by water.

\* \* \* \* \*